

**1**

3,734,759

**PROCESS FOR MAKING CARBOXYMETHYL CELLULOSE CARRIERS FOR BLUING AND FLUORESCERS**

Burton H. Gedge III, Wyoming, Ohio, assignor to The Procter & Gamble Company, Cincinnati, Ohio  
No Drawing. Filed May 20, 1971, Ser. No. 145,576  
Int. Cl. C08b 27/76

U.S. CL. 106—193

4 Claims

**ABSTRACT OF THE DISCLOSURE**

A process of producing dyed alkali metal carboxymethylcellulose via a slurry process wherein cellulose is dyed after adding it to an alkali hydroxide-solvent-water mixture and prior to reacting it with monochloroacetic acid.

**BACKGROUND OF THE INVENTION**

Slurry processes for making carboxymethylcellulose are well known in the art. U.S. Patent 2,135,128 issued to Edward Boaden Thomas et al. on Nov. 1, 1938 and U.S. Patent 2,517,577 issued to Gene D. Klug et al. on Aug. 8, 1950 both describe slurry type processes for producing carboxymethylcellulose. However, these processes do not provide a dyed carboxymethylcellulose.

A method for obtaining dyed cellulose ethers including carboxymethylcellulose is described in U.S. Patent 2,448,515 issued to William B. Carroll, Jr. on Sept. 7, 1948. This patent describes a process for obtaining dyed cellulose ethers by dying the cellulose ether in its natural, solid form and thereby produce a dyed, solid cellulose ether which can then be dissolved in an alkali, Col. 1, lines 20-24. The cellulose ether preferred in this reference is the hydroxy ethyl cellulose because in order to practice the invention, the material should be insoluble in water and soluble in alkali. Carboxymethylcellulose used in detergent compositions does not satisfy those requirements. The patent further describes the use of the dyed hydroxy ethyl cellulose in the dying of fabrics which is not of concern in the present invention. Should a carboxymethylcellulose be dyed by the Carroll process for use in a detergent formulation, it must be rinsed and dried prior to any use in conjunction with either a detergent slurry or before it is mixed with a granular detergent product to remove excess dye.

A Canadian Patent 692,844 issued to Unilever in 1964 discloses a process for fixing optical brighteners to carboxymethylcellulose to readily permit their further transfer to a textile material. However, this patent merely teaches the use of an already prepared carboxymethylcellulose.

Thus, carboxymethylcellulose containing dyes or optical brighteners are well known in the art. However, the economical and convenient method of producing such dyed or optically brightened carboxymethylcellulose of this invention has not been disclosed.

The main object of this invention is to provide an improved and more economical process of producing a carboxymethylcellulose which is dyed. This is achieved by incorporating a critical dying step strategically into a known slurry process for making carboxymethylcellulose without creating additional mass transfer requirements. Another object of this invention is to select the dyes which are compatible with the above concepts.

An advantage of this invention is to eliminate a rinsing step which is required in all prior art dyed carboxymethylcellulose processes. The purpose of the rinsing step has been and is to remove the excess dye from the formed carboxymethylcellulose to prevent it from coloring a detergent slurry or staining a granular detergent product

**2**

with which it is dry mixed. It has been discovered that the separate drying and rinsing steps may be eliminated if the dye is introduced at a strategic time in the process for making carboxymethylcellulose as further described herein.

**BRIEF SUMMARY OF THE INVENTION**

The improved process for producing a dyed alkali metal carboxymethylcellulose comprises mixing an organic solvent with water, adding cellulose which is to be converted to an alkali metal carboxymethylcellulose to the mixture, subsequently reacting the cellulose, solvent, water mixtures with an aqueous solution of alkali metal hydroxide, adding the dye to be used, then acidifying the mixture by adding monochloroacetic acid. This single process achieves both conversion of and dying of the cellulose to a dyed alkali metal, e.g., sodium, carboxymethylcellulose.

The dyed alkali metal carboxymethylcellulose can then be filtered and added to a detergent slurry to be crutched and spray dried. Alternatively, the dyed cellulose can be filtered and dried and directly dry-mixed with a granular detergent composition. The product produced by this process surprisingly, does not stain either the mixture to be crutched or the already formed granular detergent compositions.

**DETAILED DESCRIPTION OF THE INVENTION**

The process of this invention for obtaining a dyed alkali metal carboxymethylcellulose product is comprised of the following steps:

- (1) mixing from about 1 to about 20 parts of an organic solvent selected from the group consisting of methyl acetate, methylethylketone, acetone, dioxane, isopropyl alcohol, tertiary butyl alcohol, and methylene ether with from about 1 to about 28 parts of water to form a solvent-water mixture;
- (2) adding from about 1 to about 20 parts of cellulose to the solvent-water mixture to form a cellulose-containing slurry;
- (3) reacting the cellulose-containing slurry with from about 0.4 to about 20 parts of an alkali metal hydroxide to form an alkalinized slurry;
- (4) adding a dye to the alkalinized slurry in an amount such that the ratio of the dye to the cellulose present in the slurry is in a range of from about 1:6 to about 1:250 to form a dye-containing slurry; and
- (5) reacting the dye-containing slurry with from about 0.4 to 2.5 moles of monochloroacetic acid per mole of cellulose whereby dyed alkali metal carboxymethylcellulose is formed.

The dyed carboxymethylcellulose has a degree of polymerization of from about 20 to about 30,000, preferably 100 to 20,000 and a degree of substitution of from about 0.4 to about 0.9, preferably 0.5 to 0.9.

The product produced by this process can be directly dry-mixed into a detergent composition or added directly to a detergent slurry to be crutched and spray-dried without the benefit of a rinsing step to remove excess dye stuffs. When the dyed carboxymethylcellulose of this invention is added to a detergent slurry before spray drying, it is virtually impossible to distinguish dyed carboxymethylcellulose granules from the remainder of the detergent granules produced after the slurry is spray-dried. Thus, by practicing the present invention, it is possible to provide a detergent composition containing bluing ingredients or optical brighteners which are not visible to the naked eye. Such a product provides flexibility in the formulation of detergent compositions.

The organic solvent used in this process can be selected from the group consisting of methylacetate, methylethyl-

ketone, acetone, dioxane, isopropyl alcohol, tertiary butyl alcohol, and methylene ether, or mixtures of these solvents. In the practice of the invention, purified cellulose, for example, chemical cellulose prepared from wood or cotton linters as dissolving grade cellulose can be used. While fibrous cellulose can be agitated to form a well dispersed slurry wherein cellulose is intimately contacted with chemical reagents, those skilled in the chemical arts will realize that contact is improved by reducing the size of cellulose particles to achieve greater particle surface area. Accordingly, it is preferred to use dissolving grade cellulose cutter ground to permit it to pass through a Tyler Standard screen of about 20 to about 60 mesh, but the beneficial results of the present process can be obtained with fibrous cellulose or with cellulose comminuted to pass screens having still smaller openings than those mentioned above.

The alkali metal hydroxide can be sodium hydroxide, potassium hydroxide or lithium hydroxide, added preferably as an aqueous solution, sodium hydroxide is the preferred hydroxide.

In the selection of the dye used to practice this invention, three factors are of importance. First the color desired in the final product, secondly, the dyes substantivity to carboxymethylcellulose, and finally, the ability of the dye to withstand the rigors of the chemical reagents to which it must be subjected to convert the cellulose to carboxymethylcellulose. The ratio of the dye to the cellulose in the slurry is in a range of from 1:6 to about 1:250, preferably from 1:10 to 1:150.

Dyed carboxymethylcellulose of this invention to be used in a granular laundry detergent should be blue or optically active to produce a white or blue-white appearing wash or both. Suitable and representative dyes which are substantive to carboxymethylcellulose and can withstand the alkali hydroxide solution to which they are initially added and the rigors of the addition of monochloroacetic acid used to form a sodium carboxymethylcellulose are listed below with references to the color index published by the American Association of Textile Chemists and Colorists, Lowell Technological Institute, Lowell, Mass. In the case of the blue dyes recommended:

Besides producing dyed carboxymethylcelluloses the present invention is also useful for making optically brightened carboxymethylcelluloses. For such an embodiment, it is only necessary to replace the aforementioned dyes with a suitable chemically resistant optical brightener. Flexibility is provided also by employing both a dye and an optical brightener simultaneously.

The optical brighteners useful in the practice of the invention are those brighteners whose brightening action is not diminished by the chloroacetic acid used in the slurry process. A satisfactory and representative brightener is marketed under the trade name Tinopal, by Geigy Chemical Corporation. The chemical name of this brightener is sodium 4(2H-naphtho(1,2-d)triazol-2-yl)-2-stilbene sulfonate. For purposes of this invention the term "fluorescers" is synonymous with optical brighteners and the term "dye" is used generically to include bluing dyes as well as optical brighteners.

#### Example I

The preferred process of this invention can be practiced as follows. One hundred five pounds of comminuted wood cellulose cut to pass a 30-mesh screen containing five pounds of water is introduced into a reactor. An aqueous acetone solution containing 2,083 pounds of acetone and 358 pounds of water is simultaneously introduced into the same reactor. The resulting slurry of comminuted cellulose in aqueous acetone is then vigorously agitated. Next, 108 pounds of an aqueous solution containing 50% of sodium hydroxide are added over a period of 0.167 hour while continuing the agitation. The total liquid to cellulose ratio in the first step reactor is 25 to 1, while the water to cellulose ratio is about 4.17 to 1 and the acetone to water ratio is about 5 to 1. The reaction slurry is maintained at a temperature of 25° C., and the slurry is stirred vigorously for 0.25 hour to alkalize the cellulose. Following the alkalization period, 1,360 pounds of liquor containing 190 pounds of water are removed from the reactor before dropping the resulting slurry of alkali cellulose into a second step reactor. One thousand two hundred two pounds of anhydrous acetone are added



These blue dyes are representative of the dyes commercially available for use in this invention.

to the second step reactor while maintaining vigorous agitation in the reactor. During the second addition of

acetone, one pound of C.I. Direct Blue 15 of the following formula:



is added to the alkali-cellulose-acetone-water mixture. This represents a ratio of dye to cellulose of about 1:100. The resulting dye-containing slurry is then treated with 58.4 pounds of monochloroacetic acid dissolved in 158 pounds of acetone over a period of 0.25 hour. The total liquid to cellulose ratio in the second step reactor is 25 to 1 while the water to cellulose ratio is about 2.7 to 1 and the acetone to water ratio is about 10 to 1. The temperature of the vigorously agitated mixture is then raised to 70° C. and maintained at this temperature for 2.5 hours with continuing agitation to etherify the cellulose. At the end of the etherification period, the slurry is cooled to 45° C. and dropped into a separator. In the separator the dyed carboxymethylcellulose product is separated from the aqueous acetone slurry and dropped into a dryer. The resulting dried and dyed carboxymethylcellulose has a D.S. of 0.76 and is noted to be visibly free of fibers and gels when dissolved in water to a 1% concentration by weight.

The dyed carboxymethylcellulose product of Example I is especially suited for use as an anti-redeposition agent and bluing agent in detergent formulations. When added

The temperatures used in the foregoing process steps can be adjusted easily by those skilled in the art to take

into consideration materials having physical properties different from those used in Example I.

#### Example II

Another example of the process of this invention follows. One hundred five pounds of comminuted wood cellulose cut to pass a 30 mesh screen containing five pounds of water is introduced into a reactor. An aqueous acetone solution containing 1,925 pounds of acetone and 358 pounds of water is simultaneously introduced into the same reactor. The resulting slurry of comminuted cellulose in aqueous acetone is then vigorously agitated. Next, 108 pounds of an aqueous solution containing 50% of sodium hydroxide are added over a period of 0.167 hour while continuing the agitation. The total liquid to cellulose ratio in the first step reactor is 25 to 1, while the water to cellulose ratio is about 4.17 to 1 and the acetone to water ratio is about 5 to 1. The reaction slurry is maintained at a temperature of 25° C., and the slurry is stirred vigorously for 0.25 hour to alkalinize the cellulose. Following the alkalization period, one pound of C.I. Direct Blue 15 of the following formula:



to a granular detergent composition by either a dry mix process or to a detergent slurry which is to be spray dried, the dyed carboxymethylcellulose does not color the remainder of the product.

The acetone solvent used in the above process can be replaced by equal parts of methyl acetate, methylethylketone, dioxane, isopropyl alcohol, tertiary butyl alcohol and methylene ether with substantially similar results.

Similarly, the dye used in the above process can be replaced by any of the following dyes obtaining substantially similar results:



In addition to a blue dye selected from the above group, the carboxymethyl cellulose may be optically dyed by adding an optical brightener such as sodium 4(2H-naphtho-(1,2-d)triazol-2-yl)-2-stilbene sulfonate.

is added to the alkali-cellulose-acetone-water mixture.

This represents a dye to cellulose ratio of about 1:100. The resulting dye-containing slurry is then treated with 58.4 pounds of monochloroacetic acid dissolved in 158 pounds of acetone over a period of 0.25 hour. The total liquid to cellulose ratio in the second step reactor is 25 to 1 while the water to cellulose ratio is about 4.17 to 1 and the acetone to water ratio is about 5 to 1. The temperature of the vigorously agitated mixture is then raised to 70° C. and maintained at this temperature for 2.5 hours with continuing agitation of etherify the cellulose. At the end of the etherification period, the slurry is cooled to 45° C. and dropped into a separator. In the separator

the dyed carboxymethylcellulose product is separated from the aqueous acetone slurry and dropped into a dryer. The resulting dyed sodium carboxymethylcellulose is found to have a D.S. of 0.55 and is noted to be visibly free of fibers and gels when dissolved in water to a 1%

concentration by weight. The dyed carboxymethylcellulose product is useful as an anti-redeposition agent and bluing agent in detergent formulations.

A dyed sodium carboxymethylcellulose prepared by this invention which contains optical brighteners is useful to provide a surprisingly economical and convenient detergent formula that is optically brightened, contains bluing and antiredeposition agents all in a highly dispersed and usable form.

All proportions herein are by weight unless otherwise specified.

What is claimed is:

1. A process for producing dyed alkali metal carboxymethylcellulose which comprises:

- (1) mixing from about 1 to about 20 parts of an organic solvent selected from the group consisting of methyl acetate, methylethylketone, acetone, dioxane, isopropyl alcohol, tertiary butyl alcohol, and methylene ether with from about 1 to about 28 parts of water to form a solvent-water mixture;
- (2) adding from about 1 to about 20 parts of cellulose to the solvent-water mixture to form a cellulose-containing slurry;
- (3) reacting the cellulose-containing slurry with from about 0.4 to about 20 parts of an alkali metal hydroxide to form an alkalized slurry
- (4) adding a dye selected from the group consisting of

(4) sodium 4-(2H-naphtho (1,2-d)triazol-2-yl)-2-stilbene sulfonate

to the alkalized slurry of step (3) in an amount such that the ratio of the dye to the cellulose present in the slurry is in a range of from about 1:6 to about 1:250 to form a dye-containing slurry; and

(5) reacting the dye-containing slurry with from about 0.4 to 2.5 moles of monochloroacetic acid per mole of cellulose whereby dyed alkali metal carboxymethylcellulose is formed.

2. The process of claim 1 wherein the amount of dye added is in a ratio of dye to cellulose of about 1:10 to 1:150.

20 3. The process of claim 1 wherein the alkali metal is selected from the group consisting of potassium, sodium or lithium.

25 4. The process of claim 1 wherein the cellulose has a particle size which permits it to pass through a Tyler standard screen of about 20 to about 60 mesh.



and



#### References Cited

##### UNITED STATES PATENTS

- |           |         |             |       |           |
|-----------|---------|-------------|-------|-----------|
| 2,517,577 | 8/1950  | Klug et al. | ----- | 260—231   |
| 1,886,480 | 11/1932 | Haller      | ----- | 106—193 D |
| 2,448,515 | 9/1948  | Carroll     | ----- | 106—193 D |

##### OTHER REFERENCES

Chem. Abst. 57:1122 C, 1962.

THEODORE MORRIS, Primary Examiner

U.S. Cl. X.R.

106—197 C